

Oct. 29, 1935.

J. FERGUSON

**2,018,886**

## GLASS FURNACE

Filed July 13, 1934



INVENTOR.  
JOHN FERGUSON.

BY Lockwood Goldsmith & Galt

**ATTORNEY'S**

## UNITED STATES PATENT OFFICE

2,018,886

## GLASS FURNACE

John Ferguson, Indianapolis, Ind.

Application July 12, 1934, Serial No. 734,914

5 Claims. (Cl. 13—6)

This invention relates to an electric furnace which is particularly adapted for the manufacture of glass, but which is useful as well for other purposes. The principal object of the invention is to improve upon the simplicity of the construction, reliability and ease of operation of an electric furnace and the mechanism for discharging material therefrom.

One feature of the invention resides in the use of a furnace having a central discharge opening and having one of its electrodes in the form of a vertically movable plunger positioned above the discharge opening and serving both as an electrode and as a means for controlling the discharge of glass from said opening.

Another feature of the invention resides in the proportioning and arrangement of the electrodes so that graphite may be used as an electrode material without substantial discoloration of the glass. Heretofore, it has been impossible to use graphite in the manufacture of high grade glass due to the discoloring effect thereof.

Another feature of the invention resides in the construction of the electrode by means of which it is protected against chemical action in the zones of greatest chemical activity.

Other objects and features of the invention will be understood from the accompanying drawing and the following description and claims:

Fig. 1 is a central vertical section through a glass furnace constructed in accordance with the invention. Fig. 2 is a sectional view through the same taken on the line 2—2 of Fig. 1.

In the drawing, there is shown, by way of illustration, an electric furnace having a substantially flat hearth 10 with a central collecting well 11 formed in the floor thereof. A discharge opening 12 is placed in the floor of the collecting well 11. The furnace is covered by a hood 13, the apex of which communicates with a hopper 14 by means of a passage 15. Supported upon brackets 16 within the hood 13 there is a distributing cone 17 which serves to distribute the batch material 18 about the periphery of the hearth.

An outer electrode 19 consists of a plurality of arcuate blocks 20 preferably of graphite, said blocks being clamped by a two-piece metallic hoop 21 to form a circular structure adjacent the outer edge of the hearth. Arms 22 extend from the hoop 21 and are suitably insulated from the hood 13.

The central electrode consists of a plunger 23 preferably formed of graphite and supported upon the lower end of a rod 24 extending upward through a tube 25. Within the tube 25 there is

a bushing 26 of insulating material preventing electrical contact between the rod 24 and the said tube. The upper part of the graphite plunger 23 is surrounded by a shell 27 of refractory material.

The upper end of the rod 24 is pivotally connected to a lever 28 which is fulcrumed upon a bracket 29 carried by the hopper 14. The opposite end of the lever 28 is connected to the piston rod 30 of a pneumatic cylinder 31. By means 10 of this construction, the manipulation of pressure within the cylinder 31 by means of inlet and outlet pipes 32 in a well known manner serves to raise and lower the electrode 23.

Electric power for the furnace is furnished by 15 a pair of power mains 33 connected to the primary winding of a transformer 34. The secondary winding of said transformer has one terminal connected by conductors 35 to the arms 22 and the opposite terminal connected by a conductor 36 20 to the lever 28.

Communicating with the interior of the furnace there is a pipe 37 through which the gaseous products of chemical action may escape. A valve 38 in said pipe serves to control the escape 25 of said products in such manner as to preserve a super-atmospheric pressure within the furnace.

In the operation of the furnace, the batch material for manufacture of glass is placed in the hopper 14 and passes downwardly through the 30 passage 15 over the distributing cone 17 into the outer zone of the furnace. The batch is melted by electric currents passing between the electrodes and the melted glass moves continuously from the zone of the outer electrodes toward that of the 33 inner electrode. The glass which has received the longest heat treatment in the furnace is collected in the well 11 and is discharged therefrom through the opening 12. Alternate upward and downward movements of the electrode 23 provide 40 the well known gob feed by means of which successive masses of glass of the proper weight for molding various types of glass articles are discharged through the opening 12. If continuous flow feeding from the opening 12 is desired, the 45 same is controlled by placing the electrode 23 in a stationary position at the proper height to permit the desired rate of flow. This rate may then be varied as necessary by suitable movement of the electrode.

With the concentration of current usually found adjacent the electrodes of an electric furnace, it has heretofore been impossible to use graphite electrodes without a disintegration of the electrode, which produces a marked discoloration of 55

the glass. I have found, however, that if the current concentration at the electrode surface is maintained at less than ten amperes per square inch of active electrode surface that there is no appreciable disintegration of the graphite and hence no discoloration of the glass. By virtue of the design of electrodes and furnace herein illustrated wherein the entire volume of material within the outer electrode carries current, a large amount of energy can be released for melting the batch without exceeding the current concentration which would cause disintegration.

Heretofore a further disadvantage in the use of graphite as an electrode in the manufacture of glass has been the oxidation of the graphite at the high temperatures commonly employed. In the present invention this difficulty is avoided by the use of a closed furnace from which the discharge of the products of combustion is regulated to maintain a super-atmospheric pressure. In the manufacture of glass, this product of combustion is principally carbon dioxide which has no affinity for graphite. The super-atmospheric pressure maintained need be only sufficient to prevent entrance of atmospheric oxygen.

Another difficulty heretofore experienced in the use of graphite is the chemical attack thereon at the metal line or line of contact between the molten glass and the unmelted batch material. This is the zone of greatest chemical activity. The outer electrode in the present invention is completely submerged in the molten glass and, therefore, does not reach the zone of greatest chemical activity. The inner electrode is positioned at a point where normally no unmelted batch material is found and, for that reason, is substantially immune from attack. However, if the furnace is overloaded with unmelted batch or if for any reason the distributing cone 17 is not used, batch material would reach the inner electrode, which would then be in contact with the metal line. For this purpose the refractory shell 27 is supplied to protect the graphite against the extreme chemical activity at the metal line.

The foregoing description illustrates a preferred form of the invention but the details thereof may be varied by those skilled in the art without departing from the scope of the invention as defined by the appended claims.

The invention claimed is:

1. In an electric furnace, the combination of a hearth having a collecting well with a discharge opening in the floor thereof, a pair of electrodes, one of said electrodes extending into said well, electric circuits arranged to pass a current between said electrodes, and means for vertically reciprocating the last mentioned electrode to control flow of material from said discharge opening.

2. In an electric glass furnace, the combination of a hearth having a central discharge opening, a circular outer electrode adjacent the periphery thereof, a central electrode positioned above said discharge opening, said central electrode being formed of graphite, and electric circuits arranged to pass a current between said electrodes, the proportion of said central electrode and the magnitude of said current being such that the current density at said central electrode is not greater than ten amperes per 20 square inch of active electrode surface.

3. In an electric glass furnace, the combination of a hearth, a pair of electrodes, and electric circuits arranged to pass a current between said electrodes, the proportions of said electrodes and the magnitude of said current being such that the current density at either of said electrodes is not greater than ten amperes per square inch of active electrode surface, whereby graphite may be used for the electrode material without substantial discoloration of the glass.

4. In an electric glass furnace, the combination of a hearth having a central discharge opening, a circular outer electrode adjacent the periphery thereof, a central electrode positioned above said discharge opening, electric circuits arranged to pass a current between said electrodes, and means for protecting said central electrode against chemical attack at the metal line.

5. In an electric glass furnace, the combination of a hearth having a central discharge opening, a circular outer electrode adjacent the periphery thereof, a central electrode positioned above said discharge opening, electric circuits arranged to pass a current between said electrodes, and a shell of refractory material surrounding said central electrode at and above the metal line.

JOHN FERGUSON.